

No. 739,338.

PATENTED SEPT. 22, 1903.

W. T. NICHOLLS.

MANUFACTURE OF GLASS TILES.

APPLICATION FILED FEB. 20, 1901.

NO MODEL.



*Fig. 2.*



WITNESSES

J. M. Brown  
Henry McKinley

INVENTOR

William T. Nicholls.

## UNITED STATES PATENT OFFICE.

WILLIAM T. NICHOLLS, OF WELLSBURG, WEST VIRGINIA.

## MANUFACTURE OF GLASS TILES.

SPECIFICATION forming part of Letters Patent No. 739,338, dated September 22, 1903.

Application filed February 20, 1901. Serial No. 48,136. (No model.)

*To all whom it may concern:*

Be it known that I, WILLIAM T. NICHOLLS, of Wellsburg, in the county of Brooke and State of West Virginia, have invented a new and useful Improvement in the Manufacture of Glass Tiles, of which the following is a full, clear, and exact description, reference being had to the accompanying drawings, forming part of this specification, in which—

10 Figure 1 is a partial vertical section of a glass-rolling apparatus, showing the method of making my improved tile; and Fig. 2 is a perspective view of the tile itself.

My invention relates to the glass tiles which 15 are used for walls, ceilings, or floors and which have heretofore been provided with backing material applied to their rear faces, and is designed to do away with the trouble and expense of applying backing to the sheet 20 after it is formed and provide a tile with integral projections which may be cut into any size or shape desired.

In the drawings I show in Fig. 1 the manner of forming my improved tile, the glass 25 being rolled upon a table 2 by means of a roller 3, as in the usual method of forming plate-glass. The table, however, is provided with a series of indentations or grooves, which are preferably undercut, as shown at 4, so as 30 to provide angular projections 5 upon the back of the rolled sheet with flat spaces between them. The teeth are comparatively small, being shown in about full size in Fig. 1, and I have found that by forming small 35 projections of this nature separated by flat faces they do not interfere with the cutting of the glass on any desired lines. After the sheet has thus been rolled upon the table one end is lifted slightly, and the sheet is then 40 pulled endwise and upwardly in order to withdraw the projections of the glass plate from the undercut grooves of the table. The rolled

plate may then be annealed in the ordinary manner and cut up into tiles of the desired shape and size.

The glass is of course opaque, being either white or of any desired color, and in applying the tiles to the wall the undercut projections will engage the plaster and hold the tiles securely in place.

The advantages of my invention result from the rolling of the glass with projections thereon which will engage the plaster or other surfacing and hold the tile in place. These projections may be of any desired shape, but are 55 preferably undercut, as shown, so that the cement or mortar may enter the undercut portions and secure the tile in place.

The forming of the tile in the manner above stated gives a smooth front face, since the 60 top of the sheet over which the roller passes forms the front of the tiles, and the back of the rolled sheet, which is always rough, is formed with the locking projections.

Many variations may be made in the shape 65 and size of the projections, the material of the sheet, &c., without departing from my invention.

I claim—

1. The method of forming a tile which consists in rolling its front face and simultaneously molding undercut projections on its rear face, substantially as described.

2. A tile having a rolled front face and undercut molded projections on its rear face, 75 all of said projections extending in the same direction; substantially as described.

In testimony whereof I have hereunto set my hand.

WILLIAM T. NICHOLLS.

Witnesses:

J. M. BROWN,  
HENRY MCKINLEY.